

Patented Nov. 22, 1927.

1,650,275

# UNITED STATES PATENT OFFICE.

HEINRICH HOZ, WALTER BERNOLLI, AND ARTHUR LINK, OF BASEL, SWITZERLAND,  
ASSIGNORS TO THE FIRM J. R. GEIGY S. A., OF BASEL, SWITZERLAND.

## PROCESS OF DYEING AND PRINTING ACETYL CELLULOSE.

No Drawing. Original application filed March 5, 1924, Serial No. 697,145, and in Germany March 31, 1923. Divided and this application filed July 22, 1925. Serial No. 45,408.

This application is divisional of application Ser. No. 697,145.

Hitherto known processes of dyeing acetyl-cellulose have injurious effects on the fibre.

5 Through additions to the dyeing bath or through a convenient method of previous treatment mostly by the employment of saponifying alkalis or of organic solvents, or through too high a temperature in dyeing, 10 the acetyl-cellulose is prejudicially altered, so that its valuable qualities are reduced or entirely destroyed.

It has now been discovered that with a 15 large number of dyestuffs, which by themselves have only a weak affinity for acetyl-cellulose, these disadvantages can be avoided in producing the dyeing and printing of acetyl-cellulose in the presence of aryl-carboxylic acid anions. This effect can be obtained by the addition to a dye bath or printing paste of aryl-carboxylic acid compounds 20 of any kind, in the form of free acids or salts, the dyestuffs being thus brought into a form in which they are taken up by the 25 fibre at a relatively low temperature, which is quite harmless to the acetyl-cellulose. In this case, it may be advantageous to add protective colloids such as glue, gelatine, glucose, bast soap or the like, particularly with 30 dyes which show a tendency to precipitate on the addition of organic acids.

Instead of adding aryl-carboxylic acid compounds to a dye bath or printing paste, the acetyl-cellulose can be previously treated 25 with such compounds alone and afterwards, if necessary with the addition of protective colloids, dye or printed as usual with a fresh or old bath, the essential feature being always the production of the dyeing and printing in the presence of aryl-carboxylic acid anions.

In these respects, salicylic acids and their derivatives substituted by one or more oxy-, alkyl-, chloro- or nitro-groups may be suitable for the present invention.

The particular working method is shown by the following examples.

Example 1.—2% of auramine having the formula



and 2% of sodium ortho-cresotinate are separately dissolved in water and added to a dye bath after one another at about 50° C. The acetyl-cellulose is then immersed and dyed for 3/4 of an hour at 45–50° C., during which 60 the ratio of fibre to solution is 1:60. After this, washing and further treatment is effected as usual.

Example 2.—2% of Martius yellow having the formula



4% of gelatine and 2% of benzoic acid are used in the same way as Example 1. Ratio 75 of fibre to solution 1:60.

Example 3.—The acetyl-cellulose is treated for 1/2 an hour at 45° to 50° C. with a solution of 2% of 2-oxy-isophthalic acid in water, the ratio of fibre to solution being 1:60. 80 After wringing out, it is dyed in a fresh bath containing in solution 4% of gelatin and 2% of crystallized malachite green for half-an-hour at a temperature of 45 to 50° C. Ratio of fibre to solution 1:60.

The same compounds can also be used as addition to printing pastes.

What we claim is:—

1. A process for dyeing and printing acetyl-cellulose, consisting in producing the 90

dyeing and printing of finished acetyl-cellulose with coloring matters in the presence of aryl-carboxylic acid anions.

2. A process for dyeing and printing acetyl-cellulose, consisting in adding to the dyeing and printing mass a compound containing aryl-carboxylic acid anions and in

then treating finished acetyl cellulose with the mass thus prepared.

In witness whereof we have hereunto signed our names this 10th day of July, 1925.

HEINRICH HOZ.  
WALTER BERNOULLI.  
ARTHUR LINK.